

(No Model.)

L. LÉTRANGE.

PROCESS OF AND APPARATUS FOR REDUCING ZINC ORES.

No. 286,208.

Patented Oct. 9, 1883.



Fig. 3



Fig. 4



WITNESSES:

E. B. Bollin

Geo. Sinclair

INVENTOR:

Leon Létrange  
by his attorney  
Ranke, Fraser & Cornelia

# UNITED STATES PATENT OFFICE.

LEON LÉTRANGE, OF PARIS, FRANCE.

## PROCESS OF AND APPARATUS FOR REDUCING ZINC ORES.

SPECIFICATION forming part of Letters Patent No. 286,208, dated October 9, 1883.

Application filed September 13, 1881. (No model.) Patented in France June 21, 1881, No. 143,519; in Germany July 8, 1881, No. 21,775; in Belgium July 16, 1881, No. 55,187; in England July 22, 1881, No. 3,211; in Italy August 10, 1881, No. 13,258; in Sweden October 5, 1881; in Portugal October 19, 1881, No. 701, and in Austria-Hungary November 12, 1881, No. 26,461.

To all whom it may concern:

Be it known that I, LEON LÉTRANGE, a citizen of the French Republic, residing in Paris, France, have invented certain Improvements 5 in Processes of and Apparatus for Reducing Zinc Ores; and I do hereby declare that the following is a full and exact description of the invention.

I will first describe the process.

10 The purpose of the invention is to reduce zinc ores economically by the wet process, using only heat for a slight or very moderate roasting of the ores preliminary to the main process. In addition to the production of metallic zinc in a pure state, a considerable quantity of sulphuric acid is obtained. Zinc ores are generally of two kinds—blende, or the sulphuret, and calamine, or the carbonate, of zinc. In the dry process of reducing these ores blende 15 is roasted for the purpose of entirely expelling the sulphur and reducing the ore to oxide of zinc. The sulphur is all carried off in fumes, and is not only lost, but is very injurious to surrounding vegetation and animal life. Cala- 20 mine is also roasted to expel the carbonic acid and reduce the ore to an oxide. The oxide of zinc is then subjected to a high degree of heat for a long time in closed vessels, whereby about four-fifths or five-sixths of the metallic zinc in 25 the ore is obtained, and this in an impure or alloyed state. The process is very expensive, consuming double the weight of coal compared with the weight of the ore itself, and requiring skilled and costly labor.

30 35 By the wet process as improved by me, the zinc is produced quite pure. Very little heat is required. Sulphuric acid is also obtained as a commercial product, and associated metals—such as lead, silver, and copper—are readily separated and saved.

I will first describe the entire process, and then distinguish what is of my own invention.

The process is begun with blende, or a sulphuret of zinc. It is first roasted with a very 40 moderate heat—never allowed to become excessive. This mode of roasting, instead of expelling all the sulphur, merely vaporizes the excess of sulphur, which will leave the ore in

the state of a sulphate, which is soluble in water. Very little fuel is consumed in this roasting. For the purpose of economy in utilizing the sulphur which is expelled from the blende, a quantity of calamine is also roasted at the same time as the blende. This may be placed in the same roasting-oven as the blende, or in another oven or passage, into or through which the sulphur-vapors from the roasting blende pass, and thus attack the calamine ore, from which the carbon is expelled, and convert it into a sulphate also. The quantity of calamine 50 is to be sufficient to unite with the sulphur-vapors which come to it and form the required sulphate. If more calamine is at hand to be reduced than the blende will furnish sulphur for, sulphuric acid is added sufficient to convert the oxide of zinc obtained by the roasting of the calamine into a sulphate of zinc, to be subsequently reduced in the wet way. This acid is obtained as a final result of the process—ordinarily much more than enough to 55 serve for this purpose—and thus no extrinsic acid is required.

The sulphate of zinc having been obtained from the two ores together, as above described, the wet or main process will now be described 60 in connection with the description of the apparatus used. It may be here premised that the process includes the final deposition of the metal from the sulphate of zinc by a current of electricity upon zinc plates, or plates of other 65 metals, from which the deposited metal may be readily stripped, and the recovery of the sulphuric acid thereby set free from the bath.

The apparatus consists, essentially, of a series of vessels, in which the zinciferous substance is transformed into a sulphate of zinc; a motive power, which may be steam, water, or horse power; a Gramme machine, or any electrical machine capable of producing electricity by means of a motor; and a vessel or 70 series of vessels in which to precipitate the metallic zinc by means of a current of electricity.

The apparatus is substantially represented in the accompanying drawings, of which Figure 75 80 90 95 1 is a sectional elevation of the apparatus.

Fig. 2 is a plan; and Figs. 3 and 4 are illustrative diagrams, which will be referred to hereinafter.

A A' A<sup>2</sup> A<sup>3</sup> are reservoirs or vessels, preferably set in masonry and coated interiorly with bitumen or some similar substance to render them perfectly tight. These vessels are connected by means of pipes a a a a, which lead the liquid from near the bottom of one vessel 10 to the top of that adjacent, wherein the liquid stands at a little lower level. There may be any number of these connected reservoirs, either placed in a circle, as shown in Fig. 3, or side by side, as shown in Fig. 4.

15 The four reservoirs being filled with the mineral, I let flow into the first vessel, A, dilute sulphuric acid, which dissolves the oxide of zinc therein and converts it into sulphate solution. The excess of liquid then passes on 20 successively to the other vessels, A' A<sup>2</sup> A<sup>3</sup>, converting the zinc and dissolving out the sulphate, until the solution becomes saturated. By this time the oxide of zinc in the first vessel, A, is entirely converted, and the communication 25 between it and the vessel A' is cut off and the saturated sulphate solution in A drained off into a suitable reservoir, B, through one of the pipes a' a', which connect all of said vessels with said reservoir, as shown in Fig. 2.

30 The vessel A is now cleaned of the residuum and refilled with mineral, and while this is being done the acidulated liquid is allowed to flow into vessel A', in which the material is treated in precisely the same way as that in 35 the vessel A was treated, as described. Thus each vessel in succession is filled with mineral, acidulated, drained, and refilled successively. The acidulated liquid may be supplied from an elevated reservoir, R, through a pipe, a<sup>2</sup>, 40 as shown. The saturated solution of sulphate of zinc collected in the reservoir B may be filtered and purified by well-known means, so that the resultants of precipitation may be pure; but it is not absolutely essential. The 45 residuum taken from the vessels A A' A<sup>2</sup> A<sup>3</sup> may be submitted to special treatment for the recovery of the lead and silver which will usually be found in it.

C C are the reservoirs or vessels in which 50 the metallic zinc is precipitated from the sulphate solution by means of electricity. These are by preference made of wood, and lined with glass, lead, or other material which will resist the action of sulphuric acid. In these 55 vessels are placed a series of thin plates of zinc, b b, which serve as cathodes on which the zinc is precipitated. The superficies of these should be proportionate to the decomposing-power of the electric current employed 60 to obtain the best results; or the cathodes may be of copper or polished brass, from which the zinc deposit will readily detach itself. Opposite to each cathode is placed an anode, c, of carbon or other conducting material of an 65 insoluble nature, or a conducting material covered with a coating which is insoluble in the

acid. The solution of sulphate of zinc is conducted by the depending pipes d d to the bottom of the vessels C C in a manner capable of regulation as to the desired quantity, and this 70 may be effected by stop-cocks in the pipes d d. The zinc precipitated on the cathodes by the decomposition of the sulphate liberates a proportionate quantity of sulphuric acid, which, being lighter than the saturated solution of sulphate, rises to the top of the bath. This acid is led off as fast as formed by means of pipes o o, which tap the vessels at the level of the sulphate solution and discharge into a reservoir, D. The solution is fed to the baths to replace the zinc 80 as it is precipitated and removed, and by this means the level of the solution in the bath is maintained at all times nearly the same. The degree of concentration and acidity of the bath is also maintained constant. The acid in the 85 reservoir D, or so much of it as is necessary to convert the oxide of zinc into sulphate, is drawn from the said reservoir through suitable pipes into the reservoir R, from which it can be drawn as fast as wanted into the vessels A A' A<sup>2</sup> A<sup>3</sup>. 90

Sulphuret ores have been roasted in such a manner as to produce soluble sulphates, wholly or in part, and carbonates have been roasted for converting the ores into oxides. I am not 95 aware, however, that sulphurets and carbonates have been roasted simultaneously in the same or communicating chambers in such a manner that the sulphur given off from the sulphurets to form sulphates shall unite with oxides produced by the roasting of the carbonates, so as to convert both ores at once into sulphates, as in my invention. 100

I am also aware that pure metals have been 105 precipitated from sulphates in solution by electric currents; but I am not aware that metallic ores on the large scale have been first reduced to sulphates in solution, and the pure metal deposited therefrom by electric currents on metallic plates, and the sulphuric acid 110 set free in the same operation, separated, and saved in economic quantities for commercial use.

What I claim, therefore, as my invention, and desire to secure by Letters Patent, is— 115

1. In reducing zinc ores, the process of converting them into soluble sulphates, which consists in roasting the sulphuret ores of zinc and the carbonate ores of zinc simultaneously in the same or communicating chambers and producing a sulphate from the carbonate ores with the sulphur thrown off from the sulphuret ores in reducing the same to a sulphate, substantially as and for the purpose herein specified. 120

2. The process of reducing zinc ores and producing pure metallic zinc and sulphuric acid simultaneously therefrom, which consists in simultaneously roasting sulphuret ores and carbonate ores in the same or communicating chambers, and thereby converting both ores into soluble sulphates, then leaching these 130 roasted ores, and then depositing the metallic

zinc from a solution of the sulphates by electric currents on metallic plates, and drawing sulphuric acid at the same time from the solution as fast as set free by the said electric currents, substantially as and for the purpose herein specified.

3. In an apparatus employed in the reduction of zinc ores, as herein described, the combination of the series of digesting-vessels A A' A<sup>2</sup> A<sup>3</sup>, the reservoir B, the electric depositing vessel or vessels C C, and pipes connecting the vessels and reservoir, substantially as and for the purpose herein specified.

4. The combination of the series of digesting-vessels A A' A<sup>2</sup> A<sup>3</sup>, the reservoir B, the electric depositing vessel or vessels C C, the acid-reservoirs D R, and pipes connecting the said vessels and reservoirs, substantially as herein specified.

20 5. The apparatus for use in the process of reducing zinc ores, which consists, essentially, in a reservoir for the sulphate solution, a precipitating-vessel provided with suitable anodes and cathodes, a pipe provided with a regulating-cock, leading from the reservoir to near

the bottom of the precipitating-vessel, and an outlet-pipe for the freed acid, arranged in the said vessel at the desired level of the liquid therein, whereby the strength and quantity of the sulphate solution in the precipitating-vessel are maintained constant, substantially as herein specified.

30 6. The apparatus for use in the process of reducing the ores of zinc, which consists in an acid-reservoir, R, dissolving-tank with compartments A A' A<sup>2</sup> A<sup>3</sup>, pipes a, a', and a<sup>2</sup>, reservoir B for the sulphate solution, precipitating-vessels C C, provided with suitable anodes and cathodes, depending pipes d d, acid-reservoir D, and pipes o o, arranged to draw off 40 the supernatant acid from the vessels C C, all arranged to operate substantially as and for the purpose set forth.

In witness whereof I have hereunto signed my name in the presence of two subscribing 45 witnesses.

LEON LÉTRANGE.

Witnesses:

ROBT. M. HOOPER,  
CHARLES MARSHALL.